# EUROPEAN PATENT SPECIFICATION

(11) **EP 3 827 916 B1**
(45) Date of publication and mention of the grant of the patent: **24.12.2025**
(21) Application number: 20209464.5
(22) Date of filing: 24.11.2020
(51) Int. Cl.: B22F 1/052, B22F 1/054, B22F 1/065, B22F 1/068, B22F 1/10, C22C 28/00, C22C 38/06, C22C 38/10, C22C 38/14, C22C 38/16, B22F 3/087, C22C 33/02, C22C 38/00, H01F 1/057, H01F 41/02

(54) **A MANUFACTURING METHOD OF SINTERED ND-FE-B PERMANENT MAGNET**
VERFAHREN ZUR HERSTELLUNG EINES GESINTERTEN ND-FE-B-PERMANENTMAGNETEN
PROCÉDÉ DE FABRICATION D'AIMANT PERMANENT ND-FE-B FRITTÉ

(30) Priority: 28.11.2019 CN 201911194386
(43) Date of publication of application: 02.06.2021
(73) Proprietor: Yantai Dongxing Magnetic Materials Inc., Yantai City 265500 (CN)
(72) Inventor: Xiang, Chunjie, Yantai City, 265500 (CN); Peng, Zhongjie, Yantai City, 265500 (CN); Chen, Xiulei, Yantai City, 265500 (CN); Zhu, Xiaonan, Yantai City, 265500 (CN); Zhang, Qiang, Yantai City, 265500 (CN); Ding, Kaihong, Yantai City, 265500 (CN)
(74) Representative: Gulde & Partner

(56) References cited:
- EP-A1- 3 572 165
- CN-A- 1 688 000
- CN-A- 101 105 997
- CN-A- 101 178 963
- CN-A- 101 499 346
- US-A1- 2015 243 433

## Description

### BACKGROUND OF THE INVENTION

### 1. Field of the Invention

The present invention belongs to the technical field of Nd-Fe-B permanent magnets, in particular relates to a manufacturing method of sintered Nd-Fe-B permanent magnets.

### 2. Description of the Prior Art

Nd-Fe-B magnets are widely used in many technical fields like information technology, rail transit, aerospace, and so on.

With the development of high and new technologies, the demand for Nd-Fe-B magnets of low cost and having high coercivity and high temperature stability has increased dramatically in many technological fields.

How to improve the coercivity of magnets while reducing the total amount of rare earth and the heavy rare earth content is one of the research hotspots at present.

Heavy rare earth elements like Dy or Tb, which have larger magnetocrystalline anisotropy field constants, are usually added into the magnet alloy to enhance the coercive force of the magnets. However, the magnetic moment of heavy rare earth elements and iron atoms is antiferromagnetic, this will lead to a decrease of magnetic remanence and increase the production costs, which limits their application of Nd-Fe-B.

A grain boundary diffusion process, like coating the surface of the magnet with oxides or fluorides of heavy rare earth metals Dy or Tb and conducting heat treatment to form a (Nd,Dy/Tb)2Fe14B magnetically hardened layer at the grain boundary, is another way to improve coercive force of magnets. Besides, a low melting point alloy powder without heavy rare earth is used as a diffusion source to improve the distribution of the grain boundary phase, so as to improve the coercive force.

In order to improve the magnetic properties, modifying the Nd-Fe-B powder to optimize the microstructure and structure of the magnet is known. CN1110021467A refers to a method for manufacturing magnets including mixing the Nd-Fe-B powder with an organic solution containing heavy rare earth elements so that the heavy rare earth element is coated around the magnetic particles in order to control the distribution and diffusion of heavy rare earth element and to improve the magnetic properties of the magnet.

CN1110021467A refers to another manufacturing method for Nd-Fe-B magnets. A heavy rare earth suspension prepared by a multi-stage grinding process is added to the Nd-Fe-B powder by atomization injection, so that the heavy rare earth is distributed on the surface of magnetic particles and the magnetic properties are improved. However, the methods mentioned-above have much faultiness due to volatilization of organic solvent or a multistage grinding process to prepare the suspension and the processes are relatively complex.

CN1688000A, CN101105997A, CN101178963A, and CN101499346A refer to preparation methods of Nd-Fe-B magnets, where nanosized particulates are added to the alloy powder obtained by jet milling.

US 2015/0243433 A1 refers to a method for producing neodymium-iron-boron rare earth permanent magnetic materials comprising: alloy smelting using a strip casting process, coarsely pulverization by for example hydrogen decrepitation, milling by jet mill, and compaction of the powder. In the jet milling step nanosized micro powder of oxide is added in such a manner that a particle size of jet milling is decreased. Fine powder is collected by a powder filter and powder collected by a cyclone collector are mixed.

### SUMMARY OF THE INVENTION

The present invention provides a manufacturing method of sintered Nd-Fe-B permanent magnet to overcome at least some of the drawbacks mentioned-above. In the present invention, a uniformly modified coating is formed on the surface of the Nd-Fe-B powder by mechanical mixing, meanwhile, the Nd-Fe-B powder can be transformed into a circular one, and the distribution of grain boundary phase can be improved, so as to improve the coercive force of the magnet. In particular, the preparation method for improving the coercive force of a sintered Nd-Fe-B magnet is defined in claim 1 and comprises in the order the steps of:
A) preparing Nd-Fe-B alloy flakes by a strip casting process, followed by hydrogen decrepitation of the Nd-Fe-B alloy flakes and jet milling to obtain an Nd-Fe-B powder;
B) mixing Nd-Fe-B powder and an amount of 0.1 to 5wt. % of a nanoparticulate powder in a powder mixing machine to obtain a powder mixture;
C) modification of the powder mixture obtained in step B) by applying mechanical energy under inert conditions in a mechanofusion device such that the particles of the Nd-Fe-B powder are rounded and the nanoparticulate powder adheres to the particle surface of the Nd-Fe-B powder;
D) mixing in a lubricant to the modified Nd-Fe-B powder in a powder mixing machine; and
E) align pressing the modified Nd-Fe-B powder into a green body, sintering the green body, and aging of the obtained sintered Nd-Fe-B magnet.

A main aspect of the inventive process is the modification of the Nd-Fe-B powder in step C). In a suitable mixing device, i.e. a device for mechanical fusion (also known as mechanofusion), the nanoparticulate powder is adhered, maybe even embedded, into the larger particles of the Nd-Fe-B powder. This is achieved by applying mechanical energy, i.e. the system works with mechanical forces like impact and shear. During the process the particles of the Nd-Fe-B powder also rounded, i.e. the powder particles are subjected to extrusion, friction and shearing action, wherein sharp edges and corners of the powder particles are eroded. The particles of the nanoparticulate powder may be evenly distributed on the surface of Nd-Fe-B powder and form a coating layer. In other words, two sets of particles are employed and these two sets are distinguished by their average particle size. The mechanical mixing of step C) results in the formation of a shell comprised by the set of relatively smaller particles of the nanoparticulate powder around a core, comprised of the set of relatively larger particles of the Nd-Fe-B powder. Step C) thus leads to a novel powder composite material.

The Nd-Fe-B alloy flakes prepared by the strip casting process comprise:
Nd and, optionally, one or more additional rare earth metals, wherein a total amount of the rare earth metals RE is in the range of 28wt.% ≤ RE ≤ 32wt.%;
B being present in an amount of 0.8wt.% ≤ B ≤ 1.2wt%;
M being one or more of Al, Cu, Mg, Zn, Co, Ti, Zr, Nb, and Mo, wherein a total amount of M is in the range of 0wt.% ≤ M ≤ 5wt.%; and
the balance element is Fe.

Preferably, the further REs of the Nd-Fe-B powder are at least one of Pr, Dy, and Tb.

The strip casting process of step A) may be performed under inert conditions, e.g. under argon, and the melting temperature may be in the range of 1350°C to 1500°C.

The Nd-Fe-B powder obtained by step A) has an average particle size of D50 = 2.5µm to 5µm. The nanoparticulate powder may have an average particle size of D50 = 20nm to 100nm. The average particle diameter of the particles is measured by a laser diffraction device using appropriate particle size standards. Specifically, the laser diffraction device is used to determine the particle diameter distribution of the particles, and this particle distribution is used to calculate the D50 average of particle diameters.

The nanoparticulate powder comprises a metal or an oxide selected from the group consisting of Dy, Tb, Nd, Pr, Al, Cu Mg, Zn, Ti, Zr, Nb, and Mo, or a combination thereof. Preferred are Dy, Nb, Cu, Al, DyCu alloys, such as Dy₇₀Cu₃₀, PrCu alloys, such as Pr₆₈Cu₃₂, and TiO₂, and combinations thereof.

According to an embodiment, an amount of the added lubricant in step D) is in the range of 0.05 to 0.2 wt.%.

According to another embodiment, in step E) while compressing the modified Nd-Fe-B powder during the align pressing an orienting magnetic field of 1.8T to 2.5T is applied.

According to another embodiment, in step E) the green body is sintered in a vacuum furnace at a temperature in the range of 950°C to 1100°C for 6 to 12 hours.

According to another embodiment, in step E) the sintered Nd-Fe-B achieved by sintering are subjected to an aging including a first heat treatment at 850°C to 900°C for 3 to 5 hours and a second heat treatment at 460°C to 700°C for 3 to 6 hours.

The following beneficial effects may result by the process of the present invention: Nanoparticulate powder can be effectively coated on Nd-Fe-B powder under the action of mechanical force. During sintering and aging, the nanoparticulate powder at least partly fill the grain boundaries to improve the grain boundary phase distribution and strengthen the grain boundary, so as to reduce the magnetic coupling between the grains of the main phase and improve the magnetic properties.

The shape of Nd-Fe-B powder can be rounded, which is also helpful for improving the magnetic properties of magnets. Compared with a wet coating method, the dry coating method is simple and the mature reaction process is easy to control and does not require the use of organic solvents.

### BRIEF DESCRIPTION OF THE FIGURES

Figure 1 is a scanning electron microscope (SEM) image of the Nd-Fe-B magnet according to Example 1 of the present invention.
Figure 2 is a scanning electron microscope (SEM) image of the Nd-Fe-B magnet according to Comparative Example 1.

### DETAILED DESCRIPTION OF THE INVENTION

In the following, further detailed descriptions of the present invention are given. It shall be noted that the embodiments are used only to interpret the present invention and do not have any limiting effect on it.

### Example 1

The exemplary preparation method for preparing a sintered Nd-Fe-B magnet comprises the following steps:
Alloy sheets having the composition of (PrNd)₃₂CO₁Al_{0.35}Ti_{0.1}B_{1.0}Fe_{bal}(wt.%) are prepared by a strip casting process at the melting temperature of 1450°C, wherein the thickness of the alloy sheet is between 0.25mm to 0.35mm.

The alloy sheets are subjected to hydrogen decrepitation process to break the sheets into smaller pieces.

After the decrepitation process, the alloy pieces are pulverized in a jet milling process under nitrogen to prepare an alloy powder having an average particle size of about D50=2.5µm.

An amount of 0.1 wt.% nanoparticulate copper powder is added into the Nd-Fe-B powder and then mixed in a powder mixing machine (3D mixer) for 2 hours. The nanoparticulate copper powder has an average particle size of about D50=20nm.

Next, the powder mixture obtained in previous step is added to a mechanical mixing equipment (Mechanical fusing machine, Wuxi Xinguang Powder Technology Co., Ltd.). Modification of the powder mixture is performed under inert gas conditions, at a running speed of 2000 rpm for 60min, and at a temperature of 25°C.

The modification conditions are such that the powder particles are subjected to extrusion, friction and shearing action in the mechanical mixing process, wherein the sharp edges and corners of the powder particles are eroded to improve powder roundness. Meanwhile, due to the high surface activation energy, the surface of Nd-Fe-B powder particle interacts with the nanoparticulate powder, which makes the nanoparticulate powder evenly distributed on the surface of Nd-Fe-B powder, and then forms a kind of coating layer.

After the mechanical mixing process, an amount of 0.1wt. % lubricant is added into the modified Nd-Fe-B powder and mixed for 3h in a 3D mixer, wherein the addition of lubricant is to prevent oxidation and is conducive to subsequent compression.

The modified Nd-Fe-B powder is compressed into compacts under the protection of nitrogen while applying an orienting magnetic field of 1.8 T.

The compacts are subjected to a sintering step in a vacuum furnace at a temperature of 1020°C for 12 hours, then argon is pumped for rapid cooling.

Then, the sintered compacts are treated by a first heat treatment step at 850°C for 3 hours, and a second heat treatment step at 660°C for 6 hours.

### Comparative Example 1

The production was carried out in the same manner as Example 1 except that no nanoparticulate copper powder is added and no modification by a mechanical mixing process is applied:
The alloy sheets have the composition (PrNd)₃₂Co₁Al_{0.35}Cu_{0.1}Ti_{0.1}B_{1.0}Fe_{bal}(wt.%) and are prepared by a strip casting process at the melting temperature of 1450°C, wherein the thickness of the alloy sheet is between 0.25mm to 0.35mm.

The alloy sheets are subjected to hydrogen decrepitation process to break the sheets into smaller pieces.

After the decrepitation process, the alloy pieces are pulverized in a jet milling process under nitrogen to prepare an alloy powder having an average particle size of D50=2.5µm.

An amount of 0.1wt.% lubricant is added into the Nd-Fe-B powder and mixed for 3h in a 3D mixer, wherein the addition of lubricant is to prevent oxidation and is conducive to subsequent compression.

The Nd-Fe-B powder is compressed into compacts under the protection of nitrogen while applying an orienting magnetic field of 1.8 T.

The compacts are subjected to a sintering step in a vacuum furnace at a temperature of 1020°C for 12 hours, then argon is pumped in for rapid cooling.

Then, the sintered compacts are treated by a first heat treatment step at 850°C for 3 hours, and a second heat treatment step at 660°C for 6 hours.

The magnetic properties of the magnets obtained in Embodiment 1 and Comparative Example 1 are shown in Table 1.

**Table 1**

| | Br(T) | Hcj(kA/m) | (BH)m(kJ/m³) | Hk/Hcj |
|---|---|---|---|---|
| Example 1 | 1.365 | 1637 | 354 | 0.98 |
| Comparative Example 1 | 1.367 | 1441 | 355 | 0.98 |

Compared with Comparative Example 1, the coercive force of the magnet in Example 1 increases from 18.1KOe to 20.57KOe.The magnet prepared by the method described in the present invention has a higher coercive force, which is due to the fact that the nanoparticulate copper reacts with the rare earth rich phase to form the copper rich phase with low melting point during the heat treatment. The distribution of grain boundary phase is improved, which makes the main phase grains separated, thus improving the coercivity of the magnet. The modifications caused by the inventive process are also illustrated by the SEM images of Figure 1 (magnet of Example 1) and Figure 2 (magnet of Comparative Example 1).

### Example 2

The exemplary preparation method for preparing a sintered Nd-Fe-B magnet comprises the following steps:
The alloy sheets having the composition of (PrNd)_{29.5}Co₁Ga_{0.2}B_{1.0}Fe_{bal}(wt.%) are prepared by a strip casting process at the melting temperature of 1450°C, wherein the thickness of the alloy sheet is between 0.25mm to 0.35mm.

The alloy sheets are subjected to hydrogen decrepitation process to break the sheets into smaller pieces.

After the decrepitation process, the alloy powders are pulverized in a jet milling step under nitrogen to prepare an alloy powder having an average particle size of D50=4.0µm.

The nanoparticulate powders of Dy₇₀Cu₃₀ (D50=50nm) and TiO₂ (D50=20nm) are added into the Nd-Fe-B powder and then mixed in a 3D mixer for 2 hours, wherein the addition amount converted into Dy and Ti is 0.5% and 0.1% of the weight of Nd-Fe-B , respectively.

Next, the mixing powder obtained in previous step is added to a mechanical mixing equipment and injected with inert gas at a running speed of 5000 rpm for 30min under a temperature of 25°C.

After the mechanical mixing process, an amount of 0.1wt. % lubricant is added into the modified Nd-Fe-B powder and mixed for 3h in a 3D mixer.

The modified Nd-Fe-B powder is compressed into compacts under the protection of nitrogen while applying an orienting magnetic field of 1.8 T.

The compacts are subjected to a sintering step in a vacuum furnace at a temperature of 1060°C for 12 hours, then argon is pumped for rapid cooling.

Then, the sintered compacts are treated by a first heat treatment step at 850°C for 3 hours, and a second heat treatment step at 480°C for 3 hours.

### Comparative Example 2

Compared with Example 2, the mechanical mixing process of adding nanoparticulate powder is not performed in this Comparative Example, and the Nd-Fe-B magnet is prepared as follows:
The alloy sheets having the composition of (PrNd)_{29.5}Dy_{0.5}Co₁Cu_{0.1}Ga_{0.2}Ti_{0.1}B_{1.0}Fe_{bal} (wt.%) are prepared by a strip casting process at the melting temperature of 1450°C, wherein the thickness of the alloy sheet is between 0.25mm to 0.35mm.

The alloy sheets are subjected to hydrogen desorption process to break the sheets into more smaller pieces.

After the decrepitation process, the alloy powders are pulverized in a jet milling step under nitrogen to prepare an alloy powder having an average particle size of D50=4.0µm.

An amount of 0.1wt.% lubricant is added into the Nd-Fe-B powder and mixed for 3h in a 3D mixer.

The Nd-Fe-B powder is compressed into compacts under the protection of nitrogen while applying an orienting magnetic field of 1.8 T.

The compacts are subjected to a sintering step in a vacuum furnace at a temperature of 1060°C for 12 hours, then argon is pumped for rapid cooling.

Then, the sintered compacts are treated by a first heat treatment step at 850°C for 3 hours, and a second heat treatment step at 480°C for 3 hours.

The magnetic properties of the magnets obtained in Example 2 and Comparative Example 2 are shown in Table 2.

**Table 2**

| | Br(T) | Hcj(kA/m) | (BH)m(kJ/m³) | Hk/Hcj |
|---|---|---|---|---|
| Example 2 | 1.450 | 1418 | 412 | 0.98 |
| Comparative Example 2 | 1.455 | 1235 | 408 | 0.98 |

Compared with Comparative Example 2, the remanence and coercivity of magnets in Example 2 are higher. Dy₇₀Cu₃₀ powder is coated on the surface of Nd-Fe-B powder by mechanical mixing, and (Pr,Nd,Dy)₂Fe₁₄B epitaxial layer is formed on the powder surface during heat treatment, which increases the magnetic crystal anisotropy field of the magnet, thus improving the coercivity of magnets. In addition, TiO₂ with high melting point oxide plays a pinning role in grain boundary and inhibits grain growth, which is also helpful to improve the coercivity of magnets.

### Example 3

The exemplary preparation method for preparing a sintered Nd-Fe-B magnet comprises the following steps:
The alloy sheets having the composition of Nd₂₉Co₁Al_{0.1}Cu_{0.1}B_{1.0}Fe_{bal}(wt.%) are prepared by a strip casting process at the melting temperature of 1450°C, wherein the thickness of the alloy sheet is between 0.25mm to 0.35mm.

The alloy sheets are subjected to hydrogen desorption process to break the sheets into more smaller pieces.

After the decrepitation process, the alloy pieces are pulverized in a jet milling step under nitrogen to prepare an alloy powder having an average particle size of D50=4.0µm.

Amount of 0.5 wt.% nanoparticulate Dy powder (D50=50nm) and amount of 0.1 wt.% nanoparticulate Nb powder (D50=20nm) are added into the Nd-Fe-B powder and then mixed in a 3D mixer for 2 hours.

Next, the mixing powder obtained in previous step is added to a mechanical mixing equipment and injected with inert gas at a running speed of 8000 rpm for 5min under a temperature of 25°C.

After the mechanical mixing process, an amount of 0.1wt.% lubricant is added into the nano-coated Nd-Fe-B powder and mixed for 3h in a 3D mixer.

The nano-coated Nd-Fe-B powder is compressed into compacts under the protection of nitrogen while applying an orienting magnetic field of 1.8 T.

The compacts are subjected to a sintering step in a vacuum furnace at a temperature of 1070°C for 6 hours, then argon is pumped for rapid cooling.

Then, the sintered compacts are treated by a first heat treatment step at 850°C for 3 hours, and a second heat treatment step at 500°C for 3 hours.

### Comparative Example 3

Compared with Example 3, the mechanical mixing process of adding nanoparticulate powder is not performed in this comparative example, and the Nd-Fe-B magnet is prepared as follows:
The alloy sheets having the composition of Nd₂₉Dy_{0.5}Co₁Al_{0.1}Cu_{0.1}Nb₀.0B_{1.0}Fe_{bal}(wt.%) are prepared by a strip casting process at the melting temperature of 1450°C, wherein the thickness of the alloy sheet is between 0.25mm to 0.35mm.

The alloy sheets are subjected to hydrogen desorption process to break into more smaller pieces.

After the decrepitation process, the alloy powders are pulverized in a jet milling step under nitrogen to prepare an alloy powder having an average particle size of D50=4.0µm.

An amount of 0.1wt.% lubricant is added into the Nd-Fe-B powder and mixed for 3h in a 3D mixer.

The Nd-Fe-B powder is compressed into compacts under the protection of nitrogen while applying an orienting magnetic field of 1.8 T.

The compacts are subjected to a sintering step in a vacuum furnace at a temperature of 1070°C for 6 hours, then argon is pumped for rapid cooling.

Then, the sintered compacts are treated by a first heat treatment step at 850°C for 3 hours, and a second heat treatment step at 500°C for 3 hours.

The magnetic properties of the magnets obtained in embodiment 3 and Comparative Example 3 are shown in Table 3.

**Table 3**

| | Br(T) | Hcj(kA/m) | (BH)m(kJ/m³) | Hk/Hcj |
|---|---|---|---|---|
| Example 3 | 1.462 | 1314 | 416 | 0.98 |
| Comparative Example 3 | 1.461 | 1137 | 415 | 0.98 |

As shown in Table 3, the magnet prepared by the invention has higher coercivity, which indicates that the coating of Nd-Fe-B powder by mechanical mixing has a good effect.

### Example 4

The exemplary preparation method for preparing a sintered Nd-Fe-B magnet comprises the following steps:
The alloy sheets having the composition of (PrNd)_{29.8}Co_{1.5}Cu_{0.15} Ga_{0.2}Ti_{0.1}B_{1.0}Fe_{bal}(wt.%) are prepared by a strip casting process at the melting temperature of 1480°C, wherein the thickness of the alloy sheet is between 0.25mm to 0.35mm.

The alloy sheets are subjected to hydrogen desorption process to break the sheets into more smaller pieces.

After the decrepitation process, the alloy powders are pulverized in a jet milling step under nitrogen to prepare an alloy powder having an average particle size of D50=4.0µm.

An amount of 0.2 wt.% nanoparticulate Tb powder (D50=20nm) is added into the Nd-Fe-B powder and then mixed in a 3D mixer for 2 hours.

Next, the mixing powder obtained in previous step is added to a mechanical mixing equipment and injected with inert gas at a running speed of 350 rpm for 180min under a temperature of 500°C.

After the mechanical mixing process, an amount of 0.2wt.% lubricant is added into the nano-coated Nd-Fe-B powder and mixed for 3h in a 3D mixer.

The nano-coated Nd-Fe-B powder is compressed into compacts under the protection of nitrogen while applying an orienting magnetic field of 1.8 T.

The compacts are subjected to a sintering step in a vacuum furnace at a temperature of 1050°C for 12 hours, then argon is pumped for rapid cooling.

Then, the sintered compacts are treated by a first heat treatment step at 850°C for 3 hours, and a second heat treatment step at 500°C for 3 hours.

### Comparative Example 4

Compared with Example 4, the mechanical mixing process of adding nanoparticulate terbium powder is not performed in this control group, and the Nd-Fe-B magnet is prepared as follows: The alloy sheets having the composition of (PrNd)_{29.8} Tb_{0.2}Co₁Cu_{0.15}Ga_{0.2}Ti_{0.2}B_{1.0}Fe_{bal}(wt.%) are prepared by a strip casting process at the melting temperature of 1480°C, wherein the thickness of the alloy sheet is between 0.25mm to 0.35mm.

The alloy sheets are subjected to hydrogen desorption process to break the sheets into more smaller pieces.

After the decrepitation process, the alloy powders are pulverized in a jet milling step under nitrogen to prepare an alloy powder having an average particle size of D50=4.0µm.

An amount of 0.2wt.% lubricant is added into the Nd-Fe-B powder and mixed for 3h in a 3D mixer.

The Nd-Fe-B powder is compressed into compacts under the protection of nitrogen while applying an orienting magnetic field of 1.8 T.

The compacts are subjected to a sintering step in a vacuum furnace at a temperature of 1050°C for 12 hours, then argon is pumped for rapid cooling.

Then, the sintered compacts are treated by a first heat treatment step at 850°C for 3 hours, and a second heat treatment step at 500°C for 3 hours.

The magnetic properties of the magnets obtained in Embodiment 4and Comparative Example 4 are shown in Table 4.

**Table 4**

| | Br(T) | Hcj(kA/m) | (BH)m(kJ/m³) | Hk/Hcj |
|---|---|---|---|---|
| Example 4 | 1.456 | 1441 | 409 | 0.98 |
| Comparative Example 4 | 1.445 | 1262 | 399 | 0.98 |

As can be seen from Table 4, the magnets prepared by mechanically mixing modified Nd-Fe-B powder have higher magnetic properties. The terbium added by this method mostly exists in the surface layer of powder particles, so as to avoid the sharp decline of magnet Js resulting in the decrease of remanence. In addition, the rounding of Nd-Fe-B powder is also conducive to the improvement of magnetic remanence, which improves the magnetic remanence and coercivity.

### Example 5

The exemplary preparation method for preparing a sintered Nd-Fe-B magnet comprises the following steps:
The alloy sheets having the composition of (PrNd)_{29.5}CO₁Al_{0.1}Cu_{0.1}B_{1.0}Fe_{bal}(wt.%) are prepared by a strip casting process at the melting temperature of 1450°C, wherein the thickness of the alloy sheet is between 0.25mm to 0.35mm.

The alloy sheets are subjected to hydrogen desorption process to break the sheets into more smaller pieces.

After the decrepitation process, the alloy powders are pulverized in a jet milling step under nitrogen to prepare an alloy powder having an average particle size of D50=5.0µm.

An amount of 5 wt.% nanoparticulate Pr₆₈Cu₃₂ powder (D50=50nm) is added into the Nd-Fe-B powder and then mixed in a 3D mixer for 2 hours.

Next, the mixing powder obtained in previous step is added to a mechanical mixing equipment and injected with inert gas at a running speed of 500 rpm for 180min under a temperature of 300°C.

After the mechanical mixing process, an amount of 0.1wt.% lubricant is added into the nano-coated Nd-Fe-B powder and mixed for 3h in a 3D mixer.

The nano-coated Nd-Fe-B powder is compressed into compacts under the protection of nitrogen while applying an orienting magnetic field of 1.8 T.

The compacts are subjected to a sintering step in a vacuum furnace at a temperature of 950°C for 12 hours, then argon is pumped for rapid cooling.

Then, the sintered compacts are treated by a first heat treatment step at 850°C for 3 hours, and a second heat treatment step at 460°C for 3 hours.

### Comparative Example 5

Compared with Example 5, the mechanical mixing process of adding nanoparticulate Pr₆₈Cu₃₂ powder is not performed in this control group, and the Nd-Fe-B magnet is prepared as follows:
The alloy sheets having the composition of (PrNd)_{29.5}Co₁Al_{0.1}Cu_{0.1}B_{1.0}Fe_{bal}(wt.%) are prepared by a strip casting process at the melting temperature of 1450°C, wherein the thickness of the alloy sheet is between 0.25mm to 0.35mm.

The alloy sheets are subjected to hydrogen desorption process to break into more smaller pieces.

After the decrepitation process, the alloy powders are pulverized in a jet milling step under nitrogen to prepare an alloy powder having an average particle size of D50=5.0µm.

An amount of 0.1wt.% lubricant is added into the Nd-Fe-B powder and mixed for 3h in a 3D mixer.

The Nd-Fe-B powder is compressed into compacts under the protection of nitrogen while applying an orienting magnetic field of 1.8 T.

The compacts are subjected to a sintering step in a vacuum furnace at a temperature of 950°C for 12 hours, then argon is pumped for rapid cooling.

Then, the sintered compacts are treated by a first heat treatment step at 850°C for 3 hours, and a second heat treatment step at 460°C for 3 hours.

The magnetic properties of the magnets obtained in embodiment 5 and Comparative Example 5 are shown in Table 5.

**Table 5**

| | Br(T) | Hcj(kA/m) | (BH)m(kJ/m³) | Hk/Hcj |
|---|---|---|---|---|
| Example 5 | 1.392 | 1486 | 378 | 0.97 |
| Comparative Example 5 | 1.451 | 1078 | 404 | 0.97 |

As can be seen from Table 5, the coercivity of the magnet prepared by the present invention is significantly improved, but the remanence is reduced more. This is because the proportion of addition is large, which increases the total amount of rare earth in the magnet, so the remanence decreases obviously.

### Example 6

The differences with Example 1 are as follows: the rotating speed is 350r/min, the time is 180min, and the temperature is 500°C in the mechanical mixing process. The test results are shown in Table 6.

### Example 7

The differences with Example 1 are as follows: the rotating speed is 1000r/min, the time is 150min, and the temperature is 400°C in the mechanical mixing process. The test results are shown in Table 6.

### Example 8

The differences with Example 1 are as follows: the rotating speed is 4000r/min, the time is 120min, and the temperature is 300°C in the mechanical mixing process. The test results are shown in Table 6.

### Example 9

The differences with Example 1 are as follows: the rotating speed is 6000r/min, the time is 80min, and the temperature is 200°C in the mechanical mixing process. The test results are shown in Table 6.

### Comparative Example 6

The differences with Example 1 are as follows: the rotating speed is 200r/min, the time is 80min, and the temperature is 15°C in the mechanical mixing process. The test results are shown in Table 6.

**Table 6**

| | Br(T) | Hcj(kA/m) | Hk/Hcj |
|---|---|---|---|
| Example 6 | 1.366 | 1504 | 0.98 |
| Example 7 | 1.398 | 1665 | 0.98 |
| Example 8 | 1.392 | 1654 | 0.98 |
| Example 9 | 1.385 | 1652 | 0.98 |
| Comparative Example 6 | 1.353 | 1449 | 0.98 |

### Example 10

The difference from Example 1 is that the nanoparticulate powder is aluminum powder (the average particle size is 20nm, and the weight ratio to Nd-Fe-B powder is 0.1%). The test results are shown in Table 7.

### Example 11

The difference from Example 1 is that the nanoparticulate powder is Dy powder (the average particle size is 50nm, and the weight ratio to Nd-Fe-B powder is 0.1%) and Nb powder (the average particle size is 20nm, the weight ratio to Nd-Fe-B powder is 0.1%). The test results are shown in Table 7.

### Example 12

The difference from Example 1 is that the nanoparticulate powder is Pr₆₈Cu₃₂ powder (the average particle size is 50nm, and the weight ratio to Nd-Fe-B powder is 0.1%). The test results are shown in Table 7.

### Example 13

The difference from Example 1 is that the nanoparticulate powder is Dy₇₀Cu₃₀ powder (the average particle size is 50nm, and the weight ratio to Nd-Fe-B powder is 0.1%) and TiO₂ powder (the average particle size is 20nm, the weight ratio to Nd-Fe-B powder is 0.1%).. The test results are shown in Table 7.

**Table 7**

| | Br(T) | Hcj(kA/m) | Hk/Hcj |
|---|---|---|---|
| Example 10 | 1.345 | 1540 | 0.98 |
| Example 11 | 1.372 | 1676 | 0.98 |
| Example 12 | 1.360 | 1648 | 0.98 |
| Example 13 | 1.375 | 1660 | 0.98 |

## Claims

1. A preparation method for improving the coercive force of a sintered Nd-Fe-B magnet, the method comprising in the order the steps of:
A) preparing Nd-Fe-B alloy flakes by a strip casting process, followed by hydrogen decrepitation of the Nd-Fe-B alloy flakes and jet milling to obtain an Nd-Fe-B powder, wherein the Nd-Fe-B alloy flakes comprise:
Nd and, optionally, one or more additional rare earth metals, wherein a total amount of the rare earth metals RE is in the range of 28wt.% ≤ RE ≤ 32wt.%;
B being present in an amount of 0.8wt.% ≤ B ≤ 1.2wt%;
M being one or more metal selected from the group consisting of Al, Cu, Mg, Zn, Co, Ti, Zr, Nb, and Mo, wherein a total amount of M is in the range of 0wt.% ≤ M ≤ 5wt.%; and the balance element is Fe, and
wherein the Nd-Fe-B powder obtained by step A) has an average particle size of D50 = wherein the average particle size of D50 for the Nd-Fe-B powder is 2.5µm to 5µm; measured and calculated as indicated in the description;
B) mixing Nd-Fe-B powder and an amount of 0.1 to 5wt. % of a nanoparticulate powder in a powder mixing machine to obtain a powder mixture, wherein the nanoparticulate wherein the average powder has an average particle size of D50 = 20nm to 100nm, particle size of D50 for the nanoparticulate powder is measured and calculated as indicated in the description; and
wherein the nanoparticulate powder comprises a metal or an oxide selected from the group consisting of Dy, Tb, Nd, Pr, Al, Cu Mg, Zn, Ti, Zr, Nb, and Mo, or a combination thereof;
C) modification of the powder mixture obtained in step B) by applying mechanical energy under inert conditions in a mechanofusion device such that the particles of the Nd-Fe-B powder are rounded and the nanoparticulate powder adheres to the particle surface of the Nd-Fe-B powder;
D) mixing in a lubricant to the modified Nd-Fe-B powder in a powder mixing machine; and
E) align pressing the modified Nd-Fe-B powder into a green body, sintering the green body, and aging of the obtained sintered Nd-Fe-B magnet,

2. The method of claim 1, wherein an amount of the added lubricant in step D) is in the range of 0.05 to 0.2 wt.%.

3. The method of one of the preceding claims, wherein in step E) while compressing the modified Nd-Fe-B powder during the align pressing an orienting magnetic field of 1.8T to 2.5T is applied.

4. The method of one of the preceding claims, wherein in step E) the green body is sintered in a vacuum furnace at a temperature in the range of 950°C to 1100°C for 6 to 12 hours.

5. The method of one of the preceding claims, wherein in step E) the sintered Nd-Fe-B achieved by sintering are subjected to an aging including a first heat treatment at 850°C to 900°C for 3 to 5 hours and a second heat treatment at 460°C to 700°C for 3 to 6 hours.

## Patentansprüche

1. Vorbereitungsverfahren zur Verbesserung der Koerzitivkraft eines gesinterten Nd-Fe-B-Magneten, wobei das Verfahren in der angegebenen Reihenfolge die folgenden Schritte umfasst:
A) Vorbereiten von Nd-Fe-B-Legierungsflocken durch einen Bandgießprozess, gefolgt von einer Wasserstoffdekrepitation der Nd-Fe-B-Legierungsflocken und einer Strahlvermahlung, um ein Nd-Fe-B-Pulver zu erhalten, wobei die Nd-Fe-B-Legierungsflocken Folgendes umfassen:
Nd und gegebenenfalls ein oder mehrere zusätzliche Seltenerdmetalle, wobei die Gesamtmenge der Seltenerdmetalle RE im Bereich von 28 Gew.-% ≤ RE ≤ 32 Gew.-% liegt;
B, das in einer Menge von 0,8 Gew.-% ≤ B ≤ 1,2 Gew.-% vorliegt;
M, das ein oder mehrere Metalle ist, ausgewählt aus der Gruppe bestehend aus Al, Cu, Mg, Zn, Co, Ti, Zr, Nb und Mo, wobei die Gesamtmenge an M im Bereich von 0 Gew.-% ≤ M ≤ 5 Gew.-% liegt; und wobei das Gleichgewichtselement Fe ist, und
wobei das durch Schritt A) erhaltene Nd-Fe-B-Pulver eine durchschnittliche Partikelgröße von D50 = 2,5 µm bis 5 µm aufweist; wobei die durchschnittliche Partikelgröße von D50 für das Nd-Fe-B-Pulver gemessen und berechnet wird, wie in der Beschreibung angegeben;
B) Mischen von Nd-Fe-B-Pulver und einer Menge von 0,1 Gew.-% bis 5 Gew.-% eines nanopartikulären Pulvers in einer Pulvermischmaschine, um eine Pulvermischung zu erhalten, wobei das nanopartikuläre Pulver eine durchschnittliche Partikelgröße von D50 = 20 nm bis 100 nm aufweist, wobei die durchschnittliche Partikelgröße von D50 für das nanopartikuläre Pulver gemessen und berechnet wird, wie in der Beschreibung angegeben; und
wobei das nanopartikuläre Pulver ein Metall oder ein Oxid umfasst, das aus der Gruppe bestehend aus Dy, Tb, Nd, Pr, Al, Cu, Mg, Zn, Ti, Zr, Nb und Mo oder einer Kombination davon ausgewählt ist;
C) Modifizieren der in Schritt B) erhaltenen Pulvermischung durch Aufbringen mechanischer Energie unter inerten Bedingungen in einer Mechanofusionsvorrichtung, so dass die Partikel des Nd-Fe-B-Pulvers abgerundet werden und das nanopartikuläre Pulver an der Partikeloberfläche des Nd-Fe-B-Pulvers haftet;
D) Einmischen eines Schmiermittels in das modifizierte Nd-Fe-B-Pulver in einer Pulvermischmaschine; und
E) Ausrichtungspressen des modifizierten Nd-Fe-B-Pulvers zu einem Grünkörper, Sintern des Grünkörpers und Altern des erhaltenen gesinterten Nd-Fe-B-Magneten.

2. Verfahren nach Anspruch 1, wobei die Menge des in Schritt D) hinzugefügten Schmiermittels im Bereich von 0,05 Gew.-% bis 0,2 Gew.-% liegt.

3. Verfahren nach einem der vorstehenden Ansprüche, wobei in Schritt E) beim Komprimieren des modifizierten Nd-Fe-B-Pulvers während der Ausrichtungspressung ein Orientierungsmagnetfeld von 1,8T bis 2,5T aufgebracht wird.

4. Verfahren nach einem der vorstehenden Ansprüche, wobei in Schritt E) der Grünkörper in einem Vakuumofen bei einer Temperatur im Bereich von 950°C bis 1100°C für 6 bis 12 Stunden gesintert wird.

5. Verfahren nach einem der vorstehenden Ansprüche, wobei in Schritt E) das durch Sintern erzielte gesinterte Nd-Fe-B einer Alterung unterzogen wird, die eine erste Wärmebehandlung bei 850°C bis 900°C für 3 bis 5 Stunden und eine zweite Wärmebehandlung bei 460°C bis 700°C für 3 bis 6 Stunden umfasst.

## Revendications

1. Procédé de préparation pour améliorer la force coercitive d'un aimant fritté Nd-Fe-B, le procédé comprenant dans l'ordre les étapes suivantes :
A) préparer des flocons d'alliage Nd-Fe-B par un processus de coulée en bande, suivi d'une décrépitation avec l'hydrogène sur des flocons d'alliage Nd-Fe-B et d'un broyage à jet pour obtenir une poudre de Nd-Fe-B, les flocons d'alliage Nd-Fe-B comprenant :
Nd et, éventuellement, un ou plusieurs métaux des terres rares supplémentaires, une quantité totale de métaux des terres rares RE étant comprise dans une plage de28 % en poids ≤ RE ≤ 32 % en poids ;
B représentant une quantité de 0,8 % en poids ≤ B ≤ 1,2 % en poids ;
M étant un ou plusieurs métaux choisis dans le groupe constitué par Al, Cu, Mg, Zn, Co, Ti, Zr, Nb et Mo, dans lequel une quantité totale de M est dans une plage de 0 % en poids ≤ M ≤ 5 % en poids ; et l'élément restant est Fe, et
dans lequelsla poudre de Nd-Fe-B obtenue à l'étape A) a une taille moyenne des particules de D50 = 2,5 µm à 5 µm ; dans lequel la taille moyenne des particules de D50 pour la poudre de Nd-Fe-B est mesurée et calculée comme indiqué dans la description ;
B) mélanger de la poudre de Nd-Fe-B et une quantité de 0,1 à 5 % en poids d'une poudre nanoparticulaire dans une machine de mélange de poudre pour obtenir un mélange de poudre, dans lequella poudre nanoparticulaire a une taille moyenne des particules de D50 = 20 nm à 100 nm, dans lequel la taille moyenne des particules de D50 pour la poudre nanoparticulaire est mesurée et calculée comme indiqué dans la description ; et
dans lequel la poudre nanoparticulaire comprend un métal ou un oxyde choisis parmi Dy, Tb, Nd, Pr, Al, Cu, Mg, Zn, Ti, Zr, Nb et Mo, ou une combinaison de ceux-ci ;
C) modifier le mélange de poudre obtenu à l'étape B) en appliquant l'énergie mécanique sous condition inerte dans un dispositif de mécanofusion de sorte que les particules de la poudre de Nd-Fe-B soient arrondies et que la poudre nanoparticulaire adhère à la surface des particules de la poudre de Nd-Fe-B ;
D) mélanger un lubrifiant à la poudre modifiée de Nd-Fe-B dans une machine de mélange de poudre ; et
E) presser en alignant la poudre modifiée de Nd-Fe-B dans un corps vert, fritter le corps vert, et vieillir l'aimant fritté Nd-Fe-B obtenu.

2. Procédé selon la revendication 1, dans lequel une quantité de lubrifiant ajouté à l'étape D) est dans le plage de 0,05 à 0,2 % en poids.

3. Procédé selon l'une des revendications précédentes, dans lequel, à l'étape E), lors de la compression de la poudre modifiée de Nd-Fe-B pendant le pressage d'alignement, un champ magnétique d'orientation de 1,8 T à 2,5 T est appliqué.

4. Procédé selon l'une des revendications précédentes, dans lequel, à l'étape E), le corps vert est fritté dans un four sous vide à une température dans la plage de 950°C à 1100°C pendant 6 à 12 heures.

5. Procédé selon l'une des revendications précédentes, dans lequel à l'étape E) le Nd-Fe-B fritté obtenu en frittant sont soumis à un vieillissement comprenant un premier traitement thermique à 850°C à 900°C pendant 3 à 5 heures et un second traitement thermique à 460°C à 700°C pendant 3 à 6 heures.
